

Dec. 19, 1939.

S. E. SHEPPARD ET AL

2,184,023

BUFFERED PHOTOGRAPHIC EMULSION

Filed June 9, 1936

FIG. 1.

AMINO GROUPS BUFFER



FIG. 2.



FIG. 3.

H.D. EFFECT OF ACID AND BASE ON SPEED AND pH OF AN EMULSION



Samuel E. Sheppard  
Raymond H. Lambert  
INVENTORS

By *Newton A. Perrine*  
*R. Frank Smith*  
ATTORNEYS

## UNITED STATES PATENT OFFICE

2,184,023

## BUFFERED PHOTOGRAPHIC EMULSION

Samuel E. Sheppard and Raymond H. Lambert,  
Rochester, N. Y., assignors, by mesne assignments,  
to Eastman Kodak Company, Rochester,  
N. Y., a corporation of New Jersey

Application June 9, 1933, Serial No. 84,817

5 Claims.

(CL 95—7)

This invention relates to gelatins for photographic purposes and, particularly, to gelatino-silver halide emulsions containing buffering agents to maintain the hydrogen ion concentration constant.

It is known that gelatin has very poor buffering action in the region most generally used and considered most desirable in photographic emulsion manufacture. This region extends between the limits of about pH 5 to about pH 10. Both above and below these limits the natural constituents of the gelatin afford a buffering action. The photographic properties of an emulsion are in part dependent upon the hydrogen ion concentration of the emulsion. In the region desirable for photographic emulsion manufacture, a slight change in the hydrogen ion concentration of the emulsion produces a great change in the photographic sensitivity or speed of the emulsion. A slight amount of a foreign acidic or basic substance, which may enter the emulsion or which may be formed in the emulsion during storage, may, therefore, result in a loss in sensitivity or a hypersensitizing which may be either general or local. Another factor which makes the control of the hydrogen ion concentration desirable has resulted from the increased use of color sensitizing and hypersensitizing dyes which usually involve the use of a high pH. In such emulsions the pH must be controlled with a great degree of accuracy.

It is, therefore, the principal object of the present invention to provide a means for obtaining a condition of constant hydrogen ion concentration in photographic emulsions.

We have found that this condition may be brought about by incorporating in the emulsion an agent which has a buffering action in the region of pH 5 to pH 10.

In the accompanying drawing, Fig. 1 is a graph illustrating a typical titration curve for a normal photographic gelatin showing the change in pH with the addition of acid or base. Fig. 2 is a graph showing the change in speed of a gelatino-silver halide emulsion with the addition of acid or base to the emulsion. Fig. 3 is a graph showing change in speed and pH of an emulsion with the addition of acid or base to an

unbuffered emulsion and to an emulsion containing buffering agents.

The hydrogen ion concentration of a solution is expressed by "pH", which is the negative power of the hydrogen ion concentration to the base 10, or the decadic logarithm of

$$\frac{1}{\text{hydrogen ion concentration}}$$

Addition of acid to the solution increases the hydrogen ion concentration, i. e., reduces the value of pH. When acid is added to a partly neutralized solution of a weakly ionized acid, the pH change is slight. This resistance to change in the hydrogen ion concentration is termed "buffering." It is exhibited by partly neutralized weak acids and bases and also by other compounds which dissociate hydrolytically to furnish acidic or basic ions.

The pH at which neutralization of these weakly ionized compounds is half complete is termed the  $pK$  value of the compound. The subscripts  $a$  or  $b$  may be added to  $pK$  (as  $pK_a$  or  $pK_b$ ) indicating acidic or basic constants respectively. Since buffers may be mono-, di-, tri-, etc., acidic or basic, the further subscripts 1, 2, 3, etc., may be added to indicate which acid or base gives the designated  $pK$  value. In this case  $pK$  is equal to the negative logarithm of the dissociation constant for acids ( $\text{pH} = pK_a$ ) and for bases  $\text{pH} = pK_b - pK_a$ , where pH is measured electrometrically and where  $K_w = 10^{-14}$  (dissociation constant of water), at about 25° C. and  $K_w = 3 \times 10^{-14}$  at about 40° C.

In the accompanying drawing we have shown in Fig. 1 a typical titration curve for gelatin illustrating the change in pH with addition of acid or base to a solution of the gelatin. Gelatin is known to be made up of chains of condensed amino-acids in polypeptide linkage, with side-chains of ionizable amino-acids. In the region below about pH 5 the gelatin exhibits a buffering action, that is, a great increase in the amount of acid added to it results in only a slight change in the value of pH. This buffering action has been attributed to the presence of the carboxyl groups in the gelatin. In the region above about pH 8.5 a similar buffering action is noted on de-

crease of acid or increase of alkali in the gelatin solution. The buffering action at this point is thought to be due to the presence of amino-groups in the gelatin although only half as effective as in the acid region. In the region between pH 5 and pH 8.5 the slope of the curve is great, indicating that a small change in the amount of the acid or base added to the gelatin solution results in a great change in the pH value 10 of the solution.

The significance of this change in pH of gelatin, which is used to manufacture photographic emulsions, is illustrated in Fig. 2. This figure shows a curve for the change in sensitivity of a photographic emulsion, expressed as H. and D. speed, plotted against amount of acid or base added to the emulsion. It will be seen from this curve that the speed of a photographic emulsion in the region of pH 5 to pH 10 is greatly affected 20 by the addition of a small amount of acid or base to the emulsion. This alteration of speed of an emulsion is, of course, highly objectionable.

Upon the addition of a small amount of a buffering agent to the photographic emulsion, the 25 slope of the curve of Fig. 1 is materially decreased, thus showing that the addition of acid or base to the emulsion results in less change in the pH of the emulsion. As indicated in Fig. 3, A is a curve for change in speed and pH of an emulsion with addition of acid or base and will be seen to be similar to the curve shown in Fig. 1. The curve B of Fig. 3 illustrates the result of adding acid or base to a similar emulsion to which 35 a buffering agent has been added. in this case the buffering agent consisting of diethylbarbituric acid (Veronal). It will be seen that in the case of the emulsion represented by the curve B, a comparatively large amount of acidic or basic material may be added to the emulsion without 40 resulting in a great change in the pH of the emulsion. As shown in this figure, the change in pH of the emulsion with change in acid or base added to the emulsion is generally comparable to the change in speed, although the two 45 are not straight line functions.

The buffering agents which may be used according to our invention must have certain definite characteristics. The buffering action of 50 chemical compounds of sufficient solubility at a given pH depends upon their electrolytic and hydrolytic dissociation constants, on the first directly, as in the case of acids or bases, and on the second indirectly, in so far as saline compounds dissociating hydrolytically furnish basic or acidic materials or definite electrolytic dissociation constants. The choice of suitable buffers in the required region of pH 5 to pH 10 is limited to acids having  $pK_a$  values of about 5.5 to about 60 9.5 and to bases having  $pK_b$  values of about 4.5 to about 8.5.

Further requirements of the buffering agents used according to our invention are a sufficiently high water solubility so that they do not crystallize out in air-dry gelatin (water content 65 12-15%) and non-reactivity with silver halides, such as sulfiding or reducing tendencies. A further requirement is that the compounds should 70 not be colored or give colored products which would affect the clarity of the emulsion.

The following buffering agents have been found suitable for incorporation in photographic emulsions. These are listed together with their  $pK$  75 values.

#### BUFFERING AGENTS—PK VALUES

At 40° C.

|                                   | $pK_{a1}$ | $pK_{a2}$ | $pK_{b1}$ | $pK_{b2}$ | $pK_{b3}$ | 5    |
|-----------------------------------|-----------|-----------|-----------|-----------|-----------|------|
| Disodium phosphate                |           | 7.3       | 6.1       |           |           |      |
| Tricarballylic acid               |           |           |           |           | 5.9       | 6.52 |
| Triethanolamine HB                |           | 6.2       |           |           |           |      |
| Maleic acid                       |           |           |           |           |           |      |
| Diethyl barbituric acid (Veronal) | 7.6       |           |           |           |           | 10   |
| Dimethyl malonic acid             | 4.92      | 7.18      |           |           |           |      |
| Cyanuric acid                     | 6.90      |           |           |           |           |      |
| Pyromellitic acid                 | 5.05      |           |           |           |           |      |
| d-Camphoric acid                  |           | 5.1       |           |           |           |      |
| Parabanic acid                    | 5.4       |           |           |           |           |      |
| Mucic acid                        | 5.6       | 8.3       |           |           |           | 15   |
| Ethylenediamine                   |           |           |           | 4.17      | 7.10      |      |
| 2:4 dichlorophenol                | 7.50      |           |           |           |           |      |
| α-Amino-n-butyric acid            | 9.1       |           |           |           |           |      |
| Malonic acid                      |           | 5.68      |           |           |           |      |
| Trichloro phenol                  | 7.65      |           |           |           |           |      |
| Iodoso benzoic acid               | 7.70      |           |           |           |           | 20   |
| Para-hydroxy benzaldehyde         | 7.65      |           |           |           |           |      |
| Acetyl acetone                    | 8.30      |           |           |           |           |      |
| Acetonyl acetone                  | 8.90      |           |           |           |           |      |
| Phloroglucinol                    | 8.50      | ?         | ?         |           |           |      |
| Resorcinol                        | 8.5       | ?         |           |           |           |      |
| Guanidine                         |           |           |           | 4.8       |           |      |
| Allantoin                         | 8.9       |           |           |           |           | 25   |
| Dimethyl-benzylamine              |           |           |           | 4.52      |           |      |
| Taurine                           | 9.1       |           |           | ?         |           |      |
| Alpha-naphthol                    | 9.25      |           |           |           |           |      |
| Diethyl-amino-ethyl alcohol       |           |           |           | 3.82      |           |      |

At 25° C.

|                          | $pK_{a1}$ | $pK_{a2}$ | $pK_{b1}$ | $pK_{b2}$ | $pK_{b3}$ | 30 |
|--------------------------|-----------|-----------|-----------|-----------|-----------|----|
| Isopropylmalonic acid    | 2.89      | 6.5       |           |           |           | 35 |
| Diethyl malonic acid     | 2.57      | 7.2       |           |           |           |    |
| Dipropyl malonic acid    | 3.00      | 7.4       |           |           |           |    |
| Malic acid               | 3.40      | 5.1       |           |           |           |    |
| ββ-diethyl succinic acid | ?         | 6.7       |           |           |           |    |
| Guaiacol                 | 7.0       |           |           |           |           | 40 |

#### AGENTS SUITABLE FOR BUFFERING IN FOLLOWING REGIONS—PK VALUES

|                             | Less than | At   | 45   |
|-----------------------------|-----------|------|------|
| Isopropyl malonic acid      |           | 6.5  | ° C. |
| Diethyl malonic acid        |           | 7.20 | 25   |
| Dipropyl malonic acid       |           | 7.40 | 25   |
| Malic acid                  |           | 5.1  | 25   |
| ββ-diethyl succinic acid    |           | 6.70 | 25   |
| Trichloro phenol            |           | 7.65 | 40   |
| Iodoso benzoic acid         |           | 7.70 | 40   |
| Guaiacol                    |           | 7.0  | 25   |
| Para-hydroxybenzaldehyde    |           | 7.65 | 40   |
| Acetyl acetone              |           | 8.30 | 40   |
| Acetonyl acetone            |           | 8.90 | 40   |
| Phloroglucinol              |           | 8.50 | 40   |
| Resorcinol                  |           | 8.50 | 40   |
| Guanidine                   |           | 8.70 | 40   |
| Allantoin                   |           | 8.90 | 40   |
| Dimethyl-benzyl-amine       |           | 9.00 | 40   |
| Taurine                     |           | 9.10 | 40   |
| Alpha-naphthol              |           | 9.25 | 40   |
| Diethyl-amino-ethyl alcohol |           | 9.70 | 40   |

Although the compounds which may be used as buffering agents according to our invention are found to fall into a number of well-defined chemical classes, such as acids, aldehydes, alcohols, etc., some of them may be grouped in more specific classes. For example, among the polybasic organic acids are included malic acid, malonic acid, isopropyl malonic acid, diethyl malonic acid, dipropyl malonic acid, maleic acid, mucic acid, tricarballylic acid, pyromellitic acid, d-camphoric acid and ββ-diethyl succinic acid. Among the heterocyclic organic compounds there are included diethyl barbituric acid, cyanuric acid, parabanic acid and allantoin. Other compounds 70 75 80 85 90 95

listed above will also be found to fall into well known groups.

As has been stated above, not all compounds which have the required  $pK$  value and function as buffering agents are suitable for use in emulsions according to our invention. Certain compounds which would be suitable for buffers for plain gelatin layers are undesirable for use in gelatino-silver halide emulsion layers by reason of their action on the sensitive silver salt. An example of a compound of this type is a hydroxylamine hydrochloride which has a suitable  $pK$  value but which has a reducing action and which tends to hypersensitize the emulsion. Certain other compounds which are inert with respect to the silver salts are unsuitable due to the formation of colored substances. Such compounds may be used if this action is not objectionable but ordinarily these compounds are unsuitable for use in emulsions. An example of a compound of this type having a suitable  $pK$  value is para-nitrophenol.

The amount of buffering agent which may be used in the emulsion varies to some extent, particularly with respect to the compound used. We have found that a 0.01 molal solution in a 5% gelatin or emulsion solution is suitable. This amounts to 0.01 gram molecular weight per liter of a 5% solution of gelatin or emulsion, or about 0.15% of buffer based on the wet emulsion, that is, as emulsion containing 90% of water. We are not limited to the use of this amount, however. The proportion may be as low as 0.05% or as great as 1.0% of buffer based on the wet emulsion, and depending, as stated above, on the solubility. The limits, as stated before, depend to some extent on the particular compound used. Certain of the compounds may not be used in excessive amounts or they will adversely affect the photographic properties of the emulsion.

We will now refer to a number of examples of emulsions buffered according to our invention, it being understood that these examples are illustrative only.

#### Example I

To 1000 grams of a gelatino-silver halide emulsion containing 80 to 85% of water there were added 2.5 grams of maleic acid and 2.5 grams of diethyl barbituric acid. This emulsion was then titrated with 0.1 normal potassium hydroxide and on titration it was found that the emulsion was buffered in the pH range of about 5 to 10.

#### Example II

A buffer, diethyl barbituric acid, (0.4% by weight wet emulsion basis) was added to an experimental emulsion while a check was made of emulsion from the same batch. Each was adjusted to the same pH. An equal amount of acid was added to each and H. and D. speeds were obtained of the finished, coated and dried materials. The results are shown in the following table:

|                                                   | pH  | Speed |
|---------------------------------------------------|-----|-------|
| Emulsion unbuffered                               | 8.0 | 800   |
| Addition of 0.25 cc. 0.1N $H_2SO_4$ /gram gelatin | 6.7 | 590   |
| Emulsion buffered                                 | 6.0 | 800   |
| Addition of 0.25 cc. 0.1N $H_2SO_4$ /gram gelatin | 7.9 | 780   |

This result was verified on a series of tests as shown by Fig. 3 in which a buffered and an unbuffered commercial emulsion was adjusted to the same pH, then equal amounts of acid and

base were added to sets of each. H. and D. speed as well as other photographic characteristics were measured. It is quite apparent that speed is held quite constant for the buffered emulsion but the unbuffered is remarkably affected. Fog 5 was decreased in the presence of buffer.

#### Example III

As showing the buffer to have no harmful but a stabilizing effect on the coated emulsion, 10 the following example is cited.

To an ordinary gelatino-silver halide negative emulsion there was added 1.2 grams of maleic acid per liter of 5% emulsion solution. The emulsion was then titrated with 0.1 normal potassium hydroxide to a pH of 6.0 to 6.2 at which pH there was found to be little change in pH on further addition of alkali. The amount of alkali added will depend on the pH of the original emulsion mixture. A portion of this emulsion was coated on glass plates and was incubated for 72 hours at 120° F. in order to obtain an accelerated aging. The pH of the emulsion after coating was found to be about 6.24.

The incubated plates were then tested for 25 photographic sensitivity or speed, for contrast or "gamma", and for fog formation. Similar tests were made on buffered unincubated emulsions and on unbuffered emulsions both incubated and unincubated. The unbuffered emulsions 30 used for comparison had a pH of 5.72. The results obtained were as follows:

|                  | Total speed |       | Gamma-8 min. development |       | Fog-8 min. development |       | 35 |
|------------------|-------------|-------|--------------------------|-------|------------------------|-------|----|
|                  | Unbuf-      | Buf-  | Unbuf-                   | Buf-  | Unbuf-                 | Buf-  |    |
|                  | fered       | fered | fered                    | fered | fered                  | fered |    |
| Unincubated..... | 49.1        | 44.7  | 2.00                     | 2.72  | .05                    | .09   | 40 |
| Incubated.....   | 44.6        | 43.7  | 3.43                     | 2.58  | .11                    | .09   |    |

We have referred in the above examples to the "total speed" of the plates. This refers to speed or sensitivity of the plate when measured 45 by the method of Hurter and Drifford. Exposures were made in a Jones type 2-B sensitometer, and the speeds determined as  $10/i$ , where  $i$  is the inertia, that is, the point at which the straight line portion of the graph of  $D$  (density) 50 against  $\log E$  (logarithm of exposure in candle-meter-seconds) cuts the abscissa.

In order to determine the gamma or contrast the plates, exposed in this sensitometer, were 55 developed for a definite length of time in the following developer:

|                                   |             |       |
|-----------------------------------|-------------|-------|
| Water.....                        | liters..... | 2.0   |
| p-Methylaminophenol sulfate.....  | grams.....  | 3.8   |
| Sodium sulphite, desiccated.....  | do.....     | 384.0 |
| Hydroquinone.....                 | do.....     | 35.2  |
| Sodium carbonate, desiccated..... | do.....     | 192.0 |
| Potassium bromide.....            | do.....     | 20.0  |
| Water to make.....                | liters..... | 4.0   |

"Gamma" was determined in the usual way and was measured according to the H. and D. scale. As is well known, "gamma" according to this method is defined as the ratio of the density range of the negative to the range of the logarithm of the exposures producing it, that is,

$$\gamma = \frac{D_2 - D_1}{\log E_2 - \log E_1}$$

where  $D_1$  and  $D_2$  are the minimum and maximum 75

densities of the corresponding exposures  $E_1$  and  $E_2$ .

The fog of the plates was measured by determining the photographic density of the unexposed plate and is expressed as such, i. e., as a density  $D = -\log T$  where  $T$ =percentage of light transmitted.

The buffers used according to our invention may be incorporated in ordinary positive or negative 10 gelatin emulsions or in emulsions designed for special uses, such as X-ray emulsions and print-out emulsions. Various silver salts may be used as the sensitive agent, such as silver chloride, silver bromide or silver iodide.

15 The incorporation of buffering agents in gelatin is not limited to gelatins used in the direct preparation of photographic emulsions, but, to any gelatin used in contact with or in conjunction with a photographic emulsion to form a photographic sensitive layer, as specifically described in the U. S. Patent No. 2,139,767, granted December 13, 1938, to Gale F. Nadeau.

For example, it is desirable that gelatin layers, 20 in contact with the emulsion layer, viz., either above, below, or interstitial in multilayered coatings, should be at the same pH as the sensitive layer, for maximum stability thereof. Furthermore, gelatin layers applied at the back of a photographic film support, with the object of equalizing 25 the moisture or water absorption of the emulsion layer, and thereby preventing curling of the film during or after processing, should be adjusted to much the same pH state as the emulsion. This will tend to equalize the rate of water absorption 30 and change of dimensions of the emulsion layer and the backing layer, and therefore prevent distortion. Likewise, gelatin overcoating layers, such as gelatin layers coated over a sensitive emulsion 35 for the purpose of protecting the sensitive emulsion, or preventing abrasion, may advantageously

be buffered to prevent adverse action on the sensitive layer.

What we claim is:

1. A gelatino-silver halide emulsion containing per liter approximately 0.02 gram-molecular weight of an organic compound selected from the group consisting of maleic acid, malonic acid, isopropyl malonic acid, diethyl malonic acid, di-propyl malonic acid, mucic acid, malic acid, tricarballylic acid, pyromellitic acid, d-camphoric acid,  $\beta\beta$ -diethyl succinic acid, diethyl barbituric acid, cyanuric acid, parabanic acid, and allantoin. 5

2. A gelatino-silver halide emulsion containing as a buffering agent approximately 0.25% of 15 maleic acid and approximately 0.25% of diethyl barbituric acid.

3. A gelatino-silver halide emulsion containing as a buffering agent approximately 0.02 gram-molecular weight per liter of maleic acid. 20

4. A gelatino-silver halide emulsion containing as a buffering agent approximately 0.02 gram-molecular weight per liter of diethyl barbituric acid. 25

5. The method of making a buffered gelatino-silver halide emulsion having a substantially constant pH within an appreciable portion of the region pH 5.5 to pH 9.5, which comprises adjusting the pH of the emulsion to the region pH 5.5 to pH 9.5, and adding to it an organic acid selected from the group consisting of polybasic and heterocyclic acids, inert with respect to silver halides, soluble in gelatin containing at least 12% of water, and having pK values affording a buffering action in the region pH 5.5 to pH 9.5, 30 said organic acid being present in sufficient amount to buffer the emulsion in the region pH 5.5 to pH 9.5. 35

SAMUEL E. SHEPPARD.

RAYMOND H. LAMBERT. 40